

1

2,718,462

**ALUMINUM SOAPS OF MIXED ISO-OCTOIC ACIDS  
AS GELLING AGENTS FOR LIQUID HYDRO-  
CARBONS**

Leonard Cohen, Baltimore, Md.

No Drawing. Application November 1, 1954,  
Serial No. 466,242

8 Claims. (Cl. 44—7)

(Granted under Title 35, U. S. Code (1952), sec. 266)

The invention described herein may be manufactured and used by or for the Government of the United States of America for governmental purposes without the payment to me of any royalty thereon.

This invention relates to aluminum soap of mixed iso-octoic acids. More particularly, it relates to the aluminum di-acid soap of mixed iso-octoic acids. These soaps have a multitude of uses and have particular utility as thickening agents for liquid hydrocarbons. Thus, when these soaps are mixed with hydrocarbon fuels such as motor gasoline, they serve to produce the jellied gasoline used in flame throwers and fire bombs.

The mixed iso-octoic acids from which these soaps are made are obtained by the oxidation of iso-octyl alcohols, the latter in turn being produced from mixed heptenes by an oxo process reaction. The acids are largely 5, 6 and 7 carbon atoms in length with resulting 3, 2 and 1 methyl group substituents on the carbon chain respectively. The 6 and 7 carbon atom chains are usually present in the greater proportion.

A disclosure of the oxo process for preparing oxidation products from olefins together with utility for these products appears in U. S. Patent No. 2,553,364.

The aluminum di-acid soap is produced by reacting an aqueous sodium soap solution of the acid containing approximately 50% excess caustic, with an aqueous solution of an inorganic aluminum soap such as aluminum sulfate. The resulting insoluble hydroxy aluminum soap is filtered and washed free of by-product salts and dried.

*Example*

Dissolve 43 grams of C. P. sodium hydroxide in 850 ml. of water. Add 100 gram of mixed iso-octoic acids (neutral equivalent=143.5) and cool to room temperature by stirring. Slowly add 342 ml. of aluminum sulfate solution containing 137 grams of  $\text{Al}_2(\text{SO}_4)_3 \cdot 18 \text{H}_2\text{O}$ , (iron free), in a fine stream with good agitation to precipitate the aluminum soap. The aluminum soap is filtered and washed free of sulfate ion as indicated by barium chloride test solution. The soap is first dried by exposure to room atmosphere over phosphorous pentoxide in a desiccator.

The aluminum di-acid soap is precipitated in accordance with the following simplified equations:



Some mono-acid soap may precipitate concurrently in accordance with the following equation:



Because of hydrolysis the tri-acid soap  $\text{AlR}_3$  does not form, and acid in excess of that required remains as much adsorbed on the di-acid soap as indicated in the following equation:



2

In the above equations HR denotes the mixed iso-octoic acids.

The dried granular aluminum soaps when added to liquid hydrocarbons create visco-elastic gels, the consistencies of which will vary with the concentration of thickening agent employed. Such gels have been prepared in concentrations ranging from 1.0% to 4.0% by weight of salt. The gels are useful in fire bombs as well as in portable and mechanical flame throwers. The percentage of salt used, largely determines the consistency of the gel and accordingly the use to which it is put. Gel consistencies are to a lesser extent dependent upon the nature of the gasoline or hydrocarbon blend used as well as the mixing and storage conditions of the gel.

One method of determining the characteristic of a gel is by means of Gardner consistencies. These are a type of viscosity measurement and are described fully in JAN-I-711, 16 December 1948, National Military Establishment Specification. Incendiary Oils, Consistency of; Test Procedures. Section: Mobilometer Methods.

Such Gardner readings will vary from <25 for a 1% gel to about 675 for a 4% gel. Typical Gardner readings of a gel made with a hydrocarbon blend consisting of 18% benzene, 20% cyclohexane, 57% n-heptane and 5% iso-octane are as follows:

| Percent Soap in Test Solvent | Gardner Consistency grams/100 sec. |
|------------------------------|------------------------------------|
| 4                            | 430                                |
| 3                            | 230                                |
| 2                            | 40                                 |
| 1                            | <25                                |

These gels are prepared by adding the required amount of soap to the test solvent and mechanically stirring. When the soap particles have solvated and swollen sufficiently, the vortex will close around the stirrer shaft and the mixture can then be stored without settling. The Gardner consistencies were determined after storage for about 24 hours at room temperature. Similar gels were made using ordinary motor gasoline in place of the hydrocarbon mixture previously referred to.

Using from 2 to 3% of soap, the readings were as follows:

| Percent Soap in Gasoline | Gardner Consistency, grams/100 sec. |
|--------------------------|-------------------------------------|
| 2.0                      | 100                                 |
| 2.5                      | 180                                 |
| 3.0                      | 300                                 |

These Gardner consistencies serve as an indicator of the physical properties of the gel and therefore the utility for which they are suitable.

Since the characteristics of a gel suitable for a portable flame thrower differs from that required in a fire bomb as well as from that required in a mechanical flame thrower, tests were made of various gels to determine their suitability in each case. In tests with a portable flame thrower, gels were prepared from regular motor gasoline and including 1.5%, 2.0% and 2.5% aluminum salts by weight. The mixtures were stirred mechanically for 25 minutes at ambient temperature and aged about 24 hours before firing. Gardner consistencies of the fuels

were determined at the time of firing. Results of these tests are tabulated as shown below:

| Thickener Concentration, Percent | Gardner Consistency, grams/100 sec. | Ignition          | Flame Characteristics | Range, yds. |
|----------------------------------|-------------------------------------|-------------------|-----------------------|-------------|
| 1.5.....                         | <25                                 | Good.....         | Wide and bushy.....   | <50         |
| 2.0.....                         | 90                                  | do.....           | Broad rod.....        | >50         |
| 2.5.....                         | 210                                 | Fair to Poor..... | Narrow rod.....       | 50 10       |

In further tests with portable flame throwers, it was found that gels having a 1.8% content of aluminum salts were optimum in performance and gave a range of about 70 yards.

It is obvious that a formulation for this purpose is a compromise which must take into consideration the type of flame desired as well as the range and ignition properties of the gel.

Tests were also made on the gels of the present invention for service as fire bomb fuels. In this instance a heavier gel may be used since there is no need to maintain a viscosity suitable for passage through a nozzle as in a flame thrower. In this instance, 100 gallons of gasoline were made into a gel using 4% soap concentration. A fire bomb was filled with this fuel and released from a plane at a speed of 200 miles per hour from an altitude of 100 feet. The following results were noted:

Ignition—good

Fireball duration—3.5 seconds

Residual burning time—11 min., 30 seconds

Percent unburnt gel—2 to 5%

Area covered—42 x 130 yds.

Other tests on fire bomb fuels showed that soap concentrations of between 3.5% and 4.0% were practical. As in the case of portable flame throwers, the composition of a gel to be used in fire bombs must likewise be a compromise, including such factors as burning time, area covered, ability to stick to objects and other factors.

Tests were also made of the fuel in mechanized flame throwers and it was found that soap concentrations similar to those used in fire bombs were suitable. Concentration of 3.75% was found to be optimum.

In addition to the uses indicated, these gels have other

military applications such as filling for land mines and other structures calculated to impede enemy operations.

In applications such as fire bombs and land mines, soap concentrations in the vicinity of 4% are customarily employed although it is to be understood that this is not a limiting concentration and percentages up to 5 and 6% may sometimes be desirable for these applications.

This application is a continuation-in-part of application Serial No. 321,747 filed November 20, 1952.

I claim:

1. A method of gelling a liquid hydrocarbon which comprises agitating a mixture of a liquid hydrocarbon fraction with from 1% to 4% by weight of an aluminum mono and di-acid soap of mixed iso-octoic acids.
- 5 2. A method in accordance with claim 1 wherein the hydrocarbon fraction is motor gasoline.
3. A method in accordance with claim 1 wherein the mixed iso-octoic acids comprise principally methyl heptoic dimethyl hexoic and trimethyl pentoic acids.
- 20 4. A method of producing an incendiary gel which comprises agitating a mixture of a liquid hydrocarbon fraction and from about 1% to about 4% by weight of an aluminum diacid soap of a mixture of acids comprising principally methyl heptoic, dimethyl hexoic and tri-
- 25 methyl pentoic acids.
5. A gelled hydrocarbon consisting essentially of an intimate mixture of 1% to 4% of an aluminum mono and di-acid soap of mixed iso-octoic acids and a liquid hydrocarbon fraction.
- 30 6. A composition in accordance with claim 5 wherein the liquid hydrocarbon fraction is motor gasoline.
7. A composition in accordance with claim 5 wherein the mixed iso-octoic acids comprise principally methyl heptoic, dimethyl hexoic and trimethyl pentoic acids.
- 35 8. A composition in accordance with claim 7 wherein the liquid hydrocarbon fraction is motor gasoline.

#### References Cited in the file of this patent

#### UNITED STATES PATENTS

|    |           |                 |               |
|----|-----------|-----------------|---------------|
| 40 | 2,390,609 | Minich          | Dec. 11, 1945 |
|    | 2,570,990 | Southern et al. | Oct. 9, 1951  |
|    | 2,618,536 | Hunn            | Nov. 18, 1952 |
|    | 2,626,897 | Young et al.    | Jan. 27, 1953 |
|    | 2,628,202 | Allison et al.  | Feb. 10, 1953 |
|    | 2,648,694 | Mason           | Aug. 11, 1953 |